

UNITED STATES PATENT OFFICE

WINFRID HENTRICH, OF WIESDORF-ON-THE-RHINE, JOSEF HILGER, OF COLOGNE-MULHEIM, AND RUDOLF KNOCHE, OF LEVERKUSEN-ON-THE-RHINE, GERMANY, ASSIGNEES TO GENERAL ANILINE WORKS, INC., OF NEW YORK, N. Y., A CORPORATION OF DELAWARE

## UNIFORM DYEING OF VISCOSE

No Drawing. Application filed November 23, 1928, Serial No. 321,513, and in Germany December 2, 1927.

The present invention relates to uniformly dyed viscose silk of different origin.

guished by their uniformity and fastness to light.

It is known that it is very difficult to obtain even shades in the dyeing of viscose of different origin, for example of knitted artificial silk.

The invention is illustrated by the following examples, without being limited thereto:

According to the present invention, these difficulties are overcome by dyeing viscose with a secondary disazo dyestuff of the general formula:

*Example 1.*—10 parts by weight of the secondary disazo dyestuff from 4-amino-1-methylbenzene-3-sulfonic acid, 1-amino-2-ethoxy-naphthalene-6-sulfonic acid and 1-hydroxy-naphthalene-4-sulfonic acid having in its free state the following formula:



20 wherein  $R_1$  represents a radical of the benzene or naphthalene series and  $R_2$  represents a radical of an amino naphthalene sulfonic acid or an amino naphthol sulfonic acid.

are dissolved in 300 parts of hot water. Knitted viscose is dyed at 80° C. in this bath for about one hour in the presence of 20% of sodium sulfate and 2% of Monopole soap (calculated on the weight of the material). Thus a beautiful powerful blue dyeing is obtained, extremely uniform both in deep and pale shades and of very satisfactory fastness to light.

The dyeings are prepared in the usual manner as is outlined in the examples, by dissolving the dyestuffs in hot water and adding to the dye-bath Glauber's salt and Monopole soap (sulfonated castor oil), if desired with the addition of a wetting agent, for instance an alkyl-naphthalene-sulfonic acid, such as isobutyl-naphthalene-disulfonic acid. The viscose is introduced into the bath at about 30° C., then the bath is slowly heated to about

*Example 2.*—The known dyestuff from 4-amino-acetanilide-3-sulfonic acid, 1-amino-2-ethoxynaphthalene-6-sulfonic acid and 1-acetylaminio-8-hydroxynaphthalene-4-sulfonic acid having in its free state the following formula:



35

40

80°C., at which temperatures the viscose is dyed for about  $\frac{3}{4}$  to 1 hour. Then the viscose is washed and dried.

from which a dye bath is prepared as described; in the above examples dyes knitted viscose a beautiful uniform bluish green shade of satisfactory fastness to light. 90

We claim:

1. As new articles of manufacture knitted viscose dyed with a dyestuff of the general formula:

5



in which  $R_1$  stands for a radical of the benzene or naphthalene series and  $R_2$  stands for the radical of an aminonaphthalenesulfonic acid or an aminonaphtholsulfonic acid, the dyeings being distinguished by their uniformity and fastness to light.

2. As new articles of manufacture knitted viscose dyed with the dyestuff of the following formula:

25



the blue dyeings being distinguished by their uniformity and fastness to light.

30 In testimony whereof we have hereunto set our hands.

WINFRID HENTRICH. [L. S.]  
 JOSEF HILGER. [L. S.]  
 RUDOLF KNOCHE. [L. S.]

35

40

45

50

55

60

65